

## UNITED STATES PATENT OFFICE

RALPH P. DE VRIES, OF NEWTONVILLE, NEW YORK, ASSIGNOR TO LUDLUM STEEL COMPANY, OF WATERVLIET, NEW YORK, A CORPORATION OF NEW JERSEY.

## STABLE-SURFACE ALLOY STEEL

No Drawing.

Application filed January 20, 1928. Serial No. 82,808.

This invention relates to alloys of steel, and more particularly to such alloys as are known to the trade as stable-surface alloy steels.

5 The main objects of my invention are to provide an alloy steel of new composition which will be resistant to scaling action at high temperatures ranging from a low red heat to temperatures as high as 1800° F., and 10 which will be resistant in varying degrees to rusting-acids and corroding agents of various kinds. This steel may be readily forged and rolled, and when it has been thus forged and rolled, it will have good strength 15 and fair ductility.

The invention is especially useful where steels are to be used for internal combustion engine poppet valves, electrical resistance heating elements, carburizing boxes, and for 20 other purposes wherein metal is desired which will resist scaling, particularly to high temperatures.

I have discovered that copper, silicon, and aluminum may be alloyed with steel in such 25 proportions as to produce a high degree of resistance to scaling at high temperatures. It is essential that such an alloy have good physical properties as regards strength and malleability. Copper when used with silicon 30 and aluminum, in the ranges hereinafter set forth, produces in this alloy the desired amount of strength and malleability and at the same time gives to this alloy a high degree of resistance to scaling at high temperatures.

35 An alloy steel made in accordance with my invention contains silicon from 0.1% to 6.0%, aluminum from 0.1% to 6.0%, and copper from 0.5% to 5.0%. I have found that for good results the silicon and aluminum taken 40 together must never be less than 2.0%, and for best results not more than 6.1% of the total alloy. I have further discovered that when the silicon and aluminum content taken together is raised to any point above 2.5% it 45 is desirable that the amount of copper be not less than 1.0%, and when the alloy containing over 2.5% of silicon and aluminum combined is to be used, it is necessary for many purposes to add at least 3% to 4% of copper.

50 Alloys of this composition can be melted

practically carbon free but for some purposes may contain carbon as high as 1.0%. The usual amount of manganese found in tool and structural steels may be present, or slightly greater amounts up to 1.5% may be used. 51 Impurities and metalloids such as sulphur, phosphorus, etc., will be kept as low as possible. Typical examples of this alloy may be noted as having the following composition, it being understood that the iron "balance" may include the manganese, impurities and metalloids mentioned above:

| Silicon | Alumi-<br>num | Copper | Carbon | Iron     |
|---------|---------------|--------|--------|----------|
| 3.50%   | 0.50%         | 3.00%  | 0.25%  | Balance. |
| 5.00%   | 0.25%         | 1.00%  | 0.32%  | Balance. |
| 2.50%   | 1.25%         | 2.50%  | 0.46%  | Balance. |

65

Aluminum and silicon when used in the 70 highest proportions herein mentioned are known to make a very coarse grained alloy of very little strength. The copper in this alloy largely overcomes these difficulties. The advantage of this alloy is further shown by 75 the nature of the oxide film which is produced by exposing these alloys to temperatures ranging from 1400 to 1800° F. The color of the oxide film which is formed is generally bright even when exposed to sharply oxidizing 80 flames. This color adds materially to the commercial possibilities of this alloy as it gives more striking evidence of its scale resisting qualities than when an alloy becomes 85 black in color. For still further refining the grain, titanium may be added in amounts running from as low as 0.1% up to 5.0%. When titanium is added, the copper content may be as high as 10%. Where it is desired to impart to the alloy which is to be subjected 90 to high temperatures, greater strength at high temperatures, I may add tungsten or molybdenum in percentages 0.5% to 5.0%, to obtain additional strength at high temperatures.

95 Alloy steels made in accordance with my invention can be readily hardened by heating above their critical ranges and then cooling in water, oil, or air as desired. For many purposes for which this alloy steel is adapt- 100

ed, it will be desirable to vary the physical properties by heat treatment which may consist of hardening as mentioned and drawing the steel by re-heating after such hardening.

5 I claim—

- 10 1. A ferrous alloy containing from 0.5% to 5% copper; from 0.5% to 6% silicon, together with from 0.1% to 2% aluminum, and characterized by its resistance to scaling and corrosion at high temperatures.
  - 15 2. A stable surface alloy steel comprising about from 0.5 to 6% of silicon, about from 0.1 to 6% of aluminum and about from 0.5 to 5% of copper.
  - 20 3. A stable surface ferrous alloy comprising about 0.5 to 6% of silicon, about from 0.1 to 6% of aluminum, the total of the silicon and aluminum being between 2% and 6.1% and about 0.5 to 5% of copper.
  - 25 4. A stable surface ferrous alloy comprising about from 0.5 to 6% of silicon, about from 0.1 to 6% of aluminum, the total of the silicon and aluminum being between 2.5% and 6% and about 1 to 5% of copper.
  - 30 5. A stable surface ferrous alloy comprising about from 0.5 to 6% of silicon, about 0.1 to 6% of aluminum, about from 1 to 10% of copper and about 0.1 to 5% of titanium.
- 35 In testimony whereof I have signed my name to this specification.

RALPH P. DE VRIES.

35

40

45

50

55

60

65